

3,347,791

**ANTIOXIDANT COMPOSITION AND ESTER LUBRICATING OIL CONTAINING IT**  
 John W. Thompson and Thomas G. Davis, Kingsport, Tenn., assignors to Eastman Kodak Company, Rochester, N.Y., a corporation of New Jersey  
 No drawing. Filed Feb. 26, 1964, Ser. No. 347,391  
 25 Claims. (Cl. 252—33.6)

This invention relates to synthetic, ester type, lubricating oils and to the problem of protecting them from oxidative degradation, especially at temperatures greater than about 300° F.

Synthetic oils of the ester type have replaced petroleum oils in many lubricant and hydraulic fluid applications where severe service conditions are encountered. As an example, esters such as bis(2-ethylhexyl)sebacate are used almost universally as lubricating oils in aircraft turbine engines of the pure jet and prop jet types. However, under such severe service conditions, these esters as a class are very susceptible to oxidative degradation. Consequently, in formulating satisfactory jet engine lube oils from esters and the like, measures must be taken to protect these esters from oxidative degradation under these severe service conditions. One such measure is to incorporate into the oil a compound which has been found to inhibit or suppress oxidative degradation of that oil, that is, to function as an antioxidant in and for said oil.

A number of arylamines have been found to be effective antioxidants for ester type, synthetic, lubricating oils at temperatures up to about 300° F. However, these same arylamines have been found to have substantially reduced antioxidant activity or to be generally ineffective antioxidants for synthetic ester oils at temperatures above about 300° F., for example, 400—550° F., which temperatures are those expected to be encountered in the operation of military and civilian jet engines currently under development.

A problem, therefore, to which this invention provides a solution is how to maintain the effectiveness of these arylamines when they are employed in ester type synthetic lubricating oils at these higher temperatures.

This invention is based upon the discovery that alkali metal salts selected from the group consisting of alkali metal salts of carboxylic acids and alkali metal salts of hydroxy aromatic compounds, at minor concentrations relative to certain arylamine antioxidants, substantially maintain the antioxidant activity of these arylamine antioxidants in ester lube oils at these higher temperatures, and even cause various arylamines to be converted from ineffective to extremely potent antioxidants in ester lube oils at these temperatures.

In summary, this invention, broadly considered, comprises an oil composition particularly useful as a lubricant at temperatures as high as 400—550° F. The oil composition consists essentially of a synthetic ester type lube oil and dissolved therein at a protective concentration a mixture consisting essentially of an arylamine portion that consists essentially of at least one arylamine and, as a high temperature activator for the arylamine portion, at least one alkali metal salt selected from the group consisting of alkali metal salts of carboxylic acids and alkali metal salts of hydroxy aromatic compounds.

The synthetic ester type lube oil portion of the composition of this invention consists essentially of at least one ester which is normally liquid at temperatures of at least 20—25° C. Such an ester includes diesters of dibasic acids and alcohol, diesters of glycols and monobasic acids, trimethylolpropane and trimethylethane triesters, pentaerythritol tetraesters and low molecular weight polyesters

such as those resulting from the reaction of a glycol and a dibasic acid, and terminated with either a monohydric alcohol or a monobasic acid. Typical, specific, synthetic ester oils are:

- 5 2-buty1-2-ethyl-1,3-propanediol dipelargonate
- 2-ethyl-2-isobutyl-1,3-propanediol diundecanoate
- Bis(2-ethylhexyl)sebacate
- Dinonyl-2-ethyl-3-methylglutarate
- 2,2,4-trimethyl-1,3-pentanediol dipelargonate
- Bis(2,2,4-trimethylpentyl)azelate
- 2,4-dimethyl-2,4-dipropyl-1,3-cyclobutanediol diundecanoate
- 2,2,4,4,6,6-hexamethyl-1,3,5-cyclohexanetriol triheptanoate
- Trimethylethane tripelargonate
- Trimethylolpropane triheptanoate
- Pentaerythritol tetrahexanoate
- Pentaerythritol tetra(50/50 octanoate/pelargonate)
- Pentaerythritol tetra(75/25 pelargonate/2-ethylhexanoate)
- 20 Polyester of neopentyl glycol and sebacic acid, terminated with 2-ethylhexanol

In addition to at least one synthetic ester, the oil portion of the composition of this invention can also consist essentially of two or more normally liquid esters. In such event, the synthetic ester type lube oil is a blend of ester oils.

The arylamine portion of the lubricating oil composition of this invention functions as an antioxidant for the

- 25 synthetic ester type lube oil component of the composition. General types of arylamines under the concepts of this invention include, in order of preference: diphenylamines, N-phenylnaphthylamines, dinaphthylamines, phenothiazines and phenylenediamines. These arylamines are preferred in the order listed on the bases of the "dirtiness" and effectiveness involved. For example, while phenothiazine currently is used in most jet lubes, it is generally considered to be a "dirty" antioxidant, especially at higher temperatures. The phenylenediamines such as N,N'-di-2-naphthylphenylenediamines have been dirty and not of the highest effectiveness in our tests. Hence, diphenylamines and N-phenylnaphthylamines are especially preferred under the concepts of this invention. Examples of diphenylamines include: diphenylamine, N-methyldiphenylamine, p-octyldiphenylamine, p,p'-dioctyldiphenylamine, and the like. Examples of N-phenylnaphthylamines include N-phenyl-1-naphthylamines, N-phenyl-2-naphthylamines, N-(p-dodecylphenyl)-2-naphthylamine, and the like. Examples of dinaphthylamines include di-1-naphthylamine, di-2-naphthylamine, and the like. Examples of phenothiazines include phenothiazine, N-ethylphenothiazine, and the like. Examples of phenylenediamines include N,N'-di-β-naphthyl-p-phenylenediamine, N,N'-diphenyl-p-phenylenediamine, and the like. For extremely high temperature service, the arylamine preferably has substituents such as alkyl groups and the like to reduce the volatility of the arylamine.
- 30
- 35
- 40
- 45
- 50
- 55

The arylamine portion of the mixture employed in the lubricating oil composition of this invention can include two or more other arylamines. An especially preferred combination of arylamines is N-phenyl-1-naphthylamine and 5-ethyl-10,10-diphenylphenazasiline at about a 2:1 weight ratio.

- 60 The high temperature activator for the arylamine portion of the lubricating oil composition of this invention consists essentially of at least one alkali metal salt selected from the group consisting of alkali metal salts of carboxylic acids and alkali metal salts of hydroxy aromatic compounds. The alkali metal salts of carboxylic acids and alkali metal salts of hydroxy aromatic compounds include the potassium, sodium, lithium, rubidium and cesium salts of these acids and compounds.
- 65
- 70

Alkali metal salts of carboxylic acids are in general represented by the formula:



wherein M is an alkali metal radical and R is a carboxylic acid residue. Types of alkali metal salts of carboxylic acids include: alkali metal salts of monobasic acids of the formula:



wherein R' is a C<sub>1</sub>-C<sub>17</sub> hydrocarbon radical which includes saturated and unsaturated aliphatic radicals (for example, alkali metal salts of acetic acid, stearic acid and the like); dibasic acid salts of the formula:



wherein R'' is a C<sub>1</sub>-C<sub>18</sub> hydrocarbon radical which includes saturated and unsaturated aliphatic radicals (for example, alkali metal salts of oxalic acid, sebacic acid and the like); alkali metal salts of polybasic acids such as those wherein the carboxylic acid residue is obtained by polymerization of unsaturated fatty acids (for example: alkali metal salts of linoleic acid dimer and alkali metal salts of linoleic acid trimer); alkali metal salts of dibasic acid half esters of the formula:



wherein R' is a C<sub>1</sub>-C<sub>17</sub> hydrocarbon radical which includes saturated and unsaturated aliphatic radicals (for example, alkali metal salts of monoethyl adipate, of the monoctyl ester of linoleic acid trimer, and the like); alkali metal salts of carboxy terminated polyesters of 600-4,000 molecular weight, such as those obtained in the reaction of glycols with dibasic acids in stoichiometric excess; alkali metal salts of imide-amide reaction products; and alkali metal salts of cyclic carboxylic acids such as, for example, naphthenic acids and the like.

Alkali metal salts of imide-amide reaction products are made by cooking at a temperature of 190-220° C. until an acid number generally in a range from about 10 to about 150 and preferably in a range from about 25 to about 75 is obtained a mixture consisting essentially of at least one amino carboxylic acid and at least one C<sub>1</sub>-C<sub>18</sub> alkyl or C<sub>1</sub>-C<sub>18</sub> alkenyl primary amine at a mole ratio of acid to amine in a range from about 1:2 to about 1:4, whereby an imide-amide reaction product consisting essentially of imide-amide compounds is formed, neutralizing the reaction product to at least 90% of its acidity with at least one alkali metal hydroxide and then removing water plus any solvent that may be present. Examples of an amino carboxylic acid are ethylenediamine tetraacetic acid (hereinafter referred to as EDTA), iminodiacetic acid, 1,2-cyclohexanediamine tetraacetic acid, and the like. Preferred amines for the imide-amide reaction products include octylamine, 2-ethylhexylamine, dodecylamine, stearylamine, oleylamine and mixtures thereof including C<sub>12</sub>-C<sub>15</sub> t-alkyl primary amine products such as the one marketed as Primene 81-R.

Alkali metal salts of hydroxy aromatic compounds are represented by the formulae:



wherein M is an alkali metal radical, R''' is selected from the group consisting of C<sub>1</sub>-C<sub>18</sub> alkyl, C<sub>1</sub>-C<sub>18</sub> alkoxy, aryl, substituted aryl and halide radicals and n is 1-4. The alkali metal salts in this category can be derived from a wide variety of hydroxy aromatic compounds. Examples of alkali metal salts in this category include p-(C<sub>1</sub>-C<sub>18</sub> alkyl)phenols (for instance, p-nonylphenol, p-dodecyl-

phenol and the like), m-pentadecylphenol, p-methoxyphenol, 2,4-dibutylphenol, p-phenylphenol, o-octylphenol, 4-chloro-6-t-butylphenol and the like. In this connection, the phenoxide type metal salts can be prepared by dissolving in each case a selected alkali metal hydroxide in an ethanol-water mixture, adding a chemically equivalent quantity of the selected phenol, stirring and heating to remove solvent and water. Other types of alkali metal salts of hydroxide aromatic compounds include alkali metal salts of naphthols (for example, alkali metal salts of 1-phenylazo-2-naphthol and the like).

Preferred types of alkali metal salts of this invention and the order of their preference are: alkali metal salts derived from amino carboxylic acids, alkali metal salts of naphthenic acids, alkali metal salts of branched chain aliphatic monocarboxylic acids, alkali metal salts of straight chain aliphatic monocarboxylic acids, alkali metal salts of substituted phenols, alkali metal salts of carboxy terminated polyesters and alkali metal salts of dibasic acid half esters. This order of preference is based for the most part on the solubilities of these alkali metal salts in synthetic ester lubricant oils generally. In other words, the more soluble an alkali metal salt is in the ester oil portion of the composition the higher the order of its preference. Alkali metal salts of the group of carboxylic acids and hydroxy aromatic compounds, incompletely soluble initially at the desired use concentration in the ester oil portion are effective and within the scope of this invention. However, it is preferred that the alkali metal salts initially be completely soluble at the desired use concentration in the ester oil portion.

The alkali metal salt can be added as such alone or in admixture with the arylamine to the ester lube oil portion of the composition, or it can be made in situ in the ester oil portion. In the latter instance, however, it is recommended that any water of formation and solvents, which are present in the composition after formulation of the alkali metal salt, be removed, for example, by distillation.

Concentration of the arylamine portion of the ester oil composition depends on the esters employed in the oil portion and on the degree of high temperature stability desired. However, for most uses, concentration of the arylamine portion is generally in a range from about 0.2 to about 10% by weight of the ester oil portion and preferably in a range from about 0.5 to about 6% by weight of the ester oil portion.

Concentration of the alkali metal salt portion of the lubricating oil composition of this invention depends on the arylamine or arylamines employed in the composition and on the degree of high temperature activation desired. However, for most uses of the lubricating oil of this invention, the concentration of the alkali metal salt is selected to give an equivalent, total, alkali metal concentration in a general range from about 0.001 to about 0.5% by weight of the ester oil portion and preferably in a range from about 0.005 to about 0.5% by weight of the ester oil portion with the weight ratio of total equivalent, alkali metal to said arylamine antioxidant portion being in a general range from about 1:30 to about 1:1000.

The lubricating oil composition of this invention is made by admixing the components thereof preferably at 50-90° C., although lower and higher temperatures can be employed.

In some embodiments of this invention, it is preferred to admix first the arylamine portion of the composition and the alkali metal salt portion of the composition, thereby forming a stabilizer mixture, and then add the stabilizer mixture to the ester oil portion of the composition. In such embodiments, the concentration of the mixture is in a range from about 0.2 to about 10% by weight of the ester oil portion and preferably in a range from about 0.5 to about 5% by weight of the ester oil portion.

In addition to a new lubricating oil composition, this invention also provides a new antioxidant composition. This composition consists essentially of an arylamine por-

tion and an alkali metal salt portion. The arylamine portion consists essentially of at least one arylamine selected from the group consisting of diphenylamines, dianaphthylamines, phenothiazines and phenylenediamines. The alkali metal salt portion consists essentially of at least one alkali metal salt selected from the group consisting of alkali metal salts of carboxylic acids and alkali metal salts of hydroxy aromatic compounds. The types of arylamines involved in these new antioxidant compositions have already been described herein in considerable detail. Also the alkali metal salts of these new antioxidant compositions have been hereinbefore described in considerable detail. In general, the weight ratio of the alkali metal salt portion to the arylamine portion of the antioxidant composition is in a range from about 1:1000 to about 1:30.

The new antioxidant composition of this invention is made by admixing the components preferably at 50-90° C., although higher and lower temperatures can be employed.

This new antioxidant composition is particularly useful in synthetic ester oils employed as high temperature lubricants, such as those previously described herein. The recommended concentration range of this new antioxidant composition in such an oil is generally from about 0.2 to about 10% by weight of the ester oil and preferably from about 0.5 to about 5% by weight of the oil.

This invention is further illustrated by the following examples of various aspects of this invention, including specific embodiments thereof. This invention is not limited to these specific embodiments unless otherwise indicated.

#### Examples 1-17

These examples illustrate specific embodiments of an ester lube oil composition of this invention, which are based on alkali metal salts of carboxylic acids as the high temperature activators for the arylamine antioxidants employed therein.

In each of the specific embodiments of these exam-

5 ples, the ester lube oil portion of the composition is 2-butyl-2-ethyl-1,3-propanediol dipelargonate. The arylamine antioxidant is a mixture consisting essentially of N-phenyl-1-naphthylamine at a concentration of 1% by weight based on the ester and 5-ethyl-10,10-diphenylphenazasiline at a concentration of 1% by weight based on the ester. The composition (components, concentration, and equivalent alkali metal concentration) of the alkali metal salt portion of each specific embodiment of these examples is given in the following Table I. These specific embodiments are made by admixing the components at 50-90° C.

10 Table I also sets forth typical data actually obtained in testing for oxidative stability at temperatures over 300° F. samples of these specific embodiments, of the ester oil alone and of the ester oil with one or the other of the arylamine antioxidant and alkali metal salt portions present. The test employed in obtaining these data is referred to herein as the 425° F. AF Oxidation Test. 15 It is described in a paper entitled "Materials for High Temperature Jet Engine Lubricants" by H. E. Adams in WADC Technical Report 59-244 (U.S. Air Force, 1959). In this test a 250 milliliter sample of the lube oil composition is heated at 425° F. in a Pyrex test tube while 96 liters of air per hour are blown through the oil composition. Freshly polished 1 inch x 1 inch x 1/2 inch coupons of steel, copper, aluminum, titanium and silver, assembled as in Method 5308.4 of Federal Test Method Standard 791, are immersed in the oil. The tube is capped with a Pyrex fitting which allows volatile products to escape. The composition is heated in 20 hour cycles and at the end of each cycle the tube is cooled, a 10 milliliter oil sample is withdrawn for analysis and the oil lost by evaporation is replaced. Ordinarily, the test is continued for six cycles or 120 hours. The 10 milliliter specimens are analyzed for viscosity in centistokes at 100° F. (ASTM Method D445) and for acid number (ASTM Method D974). An increase in viscosity and an increase in acid number denote oxidation with the extent of oxidation being proportional to the extent of the increase in viscosity and in acid number.

TABLE I

| Example No. | Alkali Metal Salt Portion                                                                                                                                                               |                                                    |                                                                            | 425° F. AF Oxidation Test Results |                                     |          |
|-------------|-----------------------------------------------------------------------------------------------------------------------------------------------------------------------------------------|----------------------------------------------------|----------------------------------------------------------------------------|-----------------------------------|-------------------------------------|----------|
|             | Component(s)                                                                                                                                                                            | Concentration, percent by wt. of ester oil portion | Equivalent alkali metal concentration, percent by wt. of ester oil portion | Oxidation time in hours           | Viscosity in centistokes at 100° F. | Acid No. |
| 1.....      | Sodium stearate.....                                                                                                                                                                    | 0.064                                              | 0.005—Na.....                                                              | 120                               | 21.5                                | 1.6      |
| 2.....      | Sodium stearate.....                                                                                                                                                                    | 0.27                                               | 0.02—Na.....                                                               | 120                               | 18.4                                | 0.6      |
| 3.....      | Sodium propionate.....                                                                                                                                                                  | 0.04                                               | 0.01—Na.....                                                               | 120                               | 18.3                                | 0.6      |
| 4.....      | Sodium pelargonate.....                                                                                                                                                                 | 0.08                                               | 0.01—Na.....                                                               | 120                               | 19.8                                | 1.3      |
| 5.....      | Sodium oleate.....                                                                                                                                                                      | 0.13                                               | 0.01—Na.....                                                               | 120                               | 19.2                                | 1.1      |
| 6.....      | Potassium stearate.....                                                                                                                                                                 | 0.17                                               | 0.02—K.....                                                                | 120                               | 17.9                                | 0.1      |
| 7.....      | Lithium stearate.....                                                                                                                                                                   | 0.84                                               | 0.02—Li.....                                                               | 120                               | 22.2                                | 1.3      |
| 8.....      | Monopotassium salt of dimer of oleic acid.....                                                                                                                                          | 0.16                                               | 0.01—K.....                                                                | 100                               | 19.1                                | 1.7      |
| 9.....      | Potassium monoethyl adipate.....                                                                                                                                                        | 0.067                                              | 0.01—K.....                                                                | 100                               | 18.8                                | 1.1      |
| 10.....     | Potassium salt of imide-amide reaction product of Acid No. 49 and derived from EDTA and C <sub>12</sub> -C <sub>15</sub> t-alkyl primary amine mixture reacted on 1:3 mole ratio basis. | 0.25                                               | 0.01—K.....                                                                | 140                               | 17.4                                | 0.4      |
| 11.....     | Potassium salt of imide-amide reaction product of Acid No. 49 and derived from EDTA and C <sub>12</sub> -C <sub>15</sub> t-alkyl primary amine mixture reacted on 1:3 mole ratio basis. | 2.50                                               | 0.1—K.....                                                                 | 120                               | 17.2                                | 0.2      |
| 12.....     | Sodium salt of imide-amide reaction product of Acid No. 49 and derived from EDTA and C <sub>12</sub> -C <sub>15</sub> t-alkyl primary amine mixture reacted on 1:3 mole ratio basis.    | 0.25                                               | 0.01—Na.....                                                               | 100                               | 18.9                                | 1.1      |

TABLE I—Continued

| Example No. | Alkali Metal Salt Portion                                                                                                                                                                                                                                                                                                             |                                                    |                                                                            | 5° F. AF Oxidation Test Results |                                     |          |
|-------------|---------------------------------------------------------------------------------------------------------------------------------------------------------------------------------------------------------------------------------------------------------------------------------------------------------------------------------------|----------------------------------------------------|----------------------------------------------------------------------------|---------------------------------|-------------------------------------|----------|
|             | Component(s)                                                                                                                                                                                                                                                                                                                          | Concentration, percent by wt. of ester oil portion | Equivalent alkali metal concentration, percent by wt. of ester oil portion | Oxidation time in hours         | Viscosity in centistokes at 100° F. | Acid No. |
| 13.....     | Cesium salt of imide-amide reaction product of Acid No. 49 and derived from EDTA and C <sub>12</sub> -C <sub>15</sub> t-alkyl primary amine mixture reacted on 1:3 mole ratio basis.                                                                                                                                                  | 0.074                                              | 0.01—Cs.....                                                               | 40                              | 19.4                                | 2.5      |
| 14.....     | Potassium salt of imide-amide reaction product of Acid No. 141 and derived from EDTA and C <sub>12</sub> -C <sub>15</sub> t-alkyl primary amine mixture reacted on 1:2 mole ratio basis.                                                                                                                                              | 0.10                                               | 0.01—K.....                                                                | 100                             | 17.5                                | 0.5      |
| 15.....     | Potassium salt of imide-amide reaction product of Acid No. 100 and derived from EDTA and 2-ethylhexylamine reacted on 1:2 mole ratio basis.                                                                                                                                                                                           | 0.14                                               | 0.01—K.....                                                                | 100                             | 17.8                                | 0.9      |
| 16.....     | Potassium salt of imide-amide reaction product of Acid No. 42 and derived from imino diacetic acid and C <sub>12</sub> -C <sub>15</sub> t-alkyl primary amine mixture reacted on 1:2 mole ratio basis.                                                                                                                                | 0.32                                               | 0.01—K.....                                                                | 100                             | 17.6                                | 17.7     |
| 17.....     | Potassium salt of imide-amide reaction product of Acid No. 79, and derived from 1,2-cyclohexanediamine tetraacetic acid and C <sub>12</sub> -C <sub>15</sub> t-alkyl primary amine mixture reacted on 1:3 mole ratio basis.                                                                                                           | 0.174                                              | 0.01—K.....                                                                | 100                             | 17.2                                | 0.4      |
|             | Ester oil without any arylamine antioxidants and without any alkali metal salts.....                                                                                                                                                                                                                                                  |                                                    |                                                                            | 0                               | 14.32                               | 0.0      |
|             |                                                                                                                                                                                                                                                                                                                                       |                                                    |                                                                            | 20                              | 229                                 | 18.7     |
|             | Ester oils with the arylamine antioxidants and without any alkali metal salts.....                                                                                                                                                                                                                                                    |                                                    |                                                                            | 0                               | 14.88                               | 0.02     |
|             |                                                                                                                                                                                                                                                                                                                                       |                                                    |                                                                            | 20                              | 30.2                                | 6.2      |
|             |                                                                                                                                                                                                                                                                                                                                       |                                                    |                                                                            | 40                              | 59.4                                | 7.5      |
|             | Ester oil without any arylamine antioxidants but with potassium salt of imide-amide reaction product of Acid No. 49 and derived from EDTA and C <sub>12</sub> -C <sub>15</sub> t-alkyl primary amine mixture on 1:3 mole basis, the salt being at a concentration of 0.25% by weight of ester oil, representing 0.01% by weight of K. |                                                    |                                                                            | 0                               | 14.49                               | 0.04     |
|             |                                                                                                                                                                                                                                                                                                                                       |                                                    |                                                                            | 20                              | 80.9                                | 9.5      |

Thus, there are provided specific ester oil lubricant compositions having a higher degree of protection relative to oxidation degradation at high temperatures. Comparison of the test data in Table I shows that a variety of alkali metal salts of carboxylic acids are effective high temperature activators for the arylamine antioxidants employed.

#### Examples 18-22

These examples illustrate specific embodiments of the composition of this invention, which are based on alkali metal salts of hydroxy aromatic compounds.

The ester oil employed in each of these specific embodiments is 2-butyl-2-ethyl-1,3-propanediol dipelarg-

inate. The arylamine antioxidant is a mixture consisting essentially of N-phenyl-1-naphthylamine at a concentration of 1% by weight based on the ester oil and 5-ethyl-10,10-diphenylphenazasiline at a concentration of 1% based on the weight of the ester oil. The composition (components, concentration and equivalent alkali metal concentration) of the alkali metal salt portion of each specific embodiment of these examples is given in the following Table II.

These specific embodiments are made by admixing the components at 50-90° C.

Also in Table II are typical data actually obtained in testing for oxidative stability at temperatures over 300°

TABLE II

| Example No. | Alkali Metal Salt Portion                                                                                                                                                                    |                                                    |                                                                            | 425° F. AF Oxidation Test Results |                                     |          |
|-------------|----------------------------------------------------------------------------------------------------------------------------------------------------------------------------------------------|----------------------------------------------------|----------------------------------------------------------------------------|-----------------------------------|-------------------------------------|----------|
|             | Component(s)                                                                                                                                                                                 | Concentration, percent by wt. of ester oil portion | Equivalent alkali metal concentration, percent by wt. of ester oil portion | Oxidation time in hours           | Viscosity in centistokes at 100° F. | Acid No. |
| 18.....     | Potassium (p-nonyl-phenoxide).....                                                                                                                                                           | 0.065                                              | 0.01—K.....                                                                | 120                               | 16.8                                | 0.6      |
| 19.....     | Potassium (p-methoxy-phenoxide).....                                                                                                                                                         | 0.65                                               | 0.1—K.....                                                                 | 120                               | 18.7                                | 0.0      |
| 20.....     | Sodium (p-nonyl-phenoxide).....                                                                                                                                                              | 0.11                                               | 0.01—Na.....                                                               | 120                               | 19.1                                | 1.2      |
| 21.....     | Potassium (2-phenyl-4-chlorophenoxy).....                                                                                                                                                    | 0.63                                               | 0.01—K.....                                                                | 120                               | 18.3                                | 0.5      |
| 22.....     | Potassium (p-methoxy-phenoxide).....                                                                                                                                                         | 0.038                                              | 0.01—K.....                                                                | 40                                | 21.8                                | 3.0      |
|             | Ester oil without any arylamine antioxidants and without any alkali metal salts.....                                                                                                         |                                                    |                                                                            | 0                                 | 14.32                               | 0.03     |
|             |                                                                                                                                                                                              |                                                    |                                                                            | 20                                | 229                                 | 18.7     |
|             | Ester oil with the arylamine antioxidants but without any alkali metal salts.....                                                                                                            |                                                    |                                                                            | 0                                 | 14.88                               | 0.03     |
|             |                                                                                                                                                                                              |                                                    |                                                                            | 20                                | 30.2                                | 6.2      |
|             |                                                                                                                                                                                              |                                                    |                                                                            | 40                                | 59.4                                | 7.5      |
|             | Ester oil without any arylamine antioxidants but with potassium (p-nonyl-phenoxide) at a concentration of 0.065% by weight of ester oil, representing 0.01% by weight based on the oil of K. |                                                    |                                                                            | 0                                 | 14.40                               | 0.03     |
|             |                                                                                                                                                                                              |                                                    |                                                                            | 20                                | 66.2                                | 9.7      |

F. samples of these specific embodiments, of the ester oil alone and of the ester oil with one or the other of the arylamine antioxidant and alkali metal salt portion. The test employed in obtaining these data is the 425° F. AF Oxidation Test.

Thus, there are provided more, specific ester oil lubricating compositions useful at high temperatures and comprising an arylamine antioxidant portion and as a high temperature activator therefor an alkali metal salt of a hydroxy aromatic compound.

Examples 23-34

These examples illustrate specific embodiments of the ester oil composition of this invention, involving various arylamine antioxidants.

The ester oil employed in each of the specific embodiments is 2-butyl-2-ethyl-1,3-propanediol dipelargonate. The composition (components and concentration) of the arylamine antioxidant portion and of the alkali metal salt portion of each of these specific embodiments are set forth in the following Table III.

These specific embodiments are made by admixing the components thereof at 50-90° C.

Table III also includes typical data actually obtained in testing for oxidative stability at temperatures over 300° F. samples of these specific embodiments and of the ester oil containing only the specific arylamine antioxidants. The test employed in obtaining the data is the 425° F. AF Oxidation Test.

TABLE III

| Example No. | Arylamine Antioxidant Portion                                       |                                                      | Alkali Metal Salt Portion                                                                                                                                                                |                                                      |                                                                              | 425° F. AF Oxidation Test |                                     |                    |
|-------------|---------------------------------------------------------------------|------------------------------------------------------|------------------------------------------------------------------------------------------------------------------------------------------------------------------------------------------|------------------------------------------------------|------------------------------------------------------------------------------|---------------------------|-------------------------------------|--------------------|
|             | Component(s)                                                        | Concentration in percent by wt. of ester oil portion | Component(s)                                                                                                                                                                             | Concentration in percent by wt. of ester oil portion | Equivalent alkali metal concentration in percent by wt. of ester oil portion | Oxidation time in hours   | Viscosity in centistokes at 100° F. | Acid No.           |
| 23          | N-phenyl-1-naphthyl-amine.<br>5-ethyl-10,10-diphenyl-phenazasiline. | 1<br>1                                               | None.....                                                                                                                                                                                |                                                      |                                                                              | 0<br>20<br>40             | 14.8<br>30.2<br>49.4                | 0.03<br>6.2<br>7.5 |
|             | N-phenyl-1-naphthyl-amine.<br>5-ethyl-10,10-diphenyl-phenazasiline. | 1<br>1                                               | Potassium salt of imide-amide reaction product of Acid No. 49 and derived from EDTA and C <sub>12</sub> -C <sub>15</sub> t-alkyl primary amine mixture reacted on 1:3 mole ratio basis.  | 0.50                                                 | 0.02-K.....                                                                  | 120                       | 16.2                                | 0.20               |
| 24          | N-phenyl-1-naphthyl-amine.<br>5-ethyl-10,10-diphenyl-phenazasiline. | 0.5<br>0.5                                           | Potassium salt of imide-amide reaction product of Acid No. 49 and derived from EDTA and C <sub>12</sub> -C <sub>15</sub> t-alkyl primary amine mixture reacted on 1:3 mole ratio basis.  | 0.25                                                 | 0.01-K.....                                                                  | 120                       | 16.2                                | 0.00               |
|             | N-phenyl-1-naphthyl-amine.<br>5-ethyl-10,10-diphenyl-phenazasiline. | 1.5<br>0.5                                           | Potassium salt of imide-amide reaction product of Acid No. 49 and derived from EDTA and C <sub>12</sub> -C <sub>15</sub> t-alkyl primary amine mixture reacted on 1:3 mole ratio basis.  | 0.25                                                 | 0.01-K.....                                                                  | 140                       | 16.8                                | 0.40               |
| 25          | N-phenyl-1-naphthyl-amine.<br>5-ethyl-10,10-diphenyl-phenazasiline. | 2                                                    | None.....                                                                                                                                                                                |                                                      |                                                                              | 40                        | 53.4                                | 9.9                |
|             | N-phenyl-1-naphthyl-amine.                                          | 2                                                    | Potassium salt of imide-amide reaction product of Acid No. 49 and derived from EDTA and C <sub>12</sub> -C <sub>15</sub> t-alkyl primary amine mixture reacted on 1:3 molar ratio basis. | 0.25                                                 | 0.01-K.....                                                                  | 140                       | 17.41                               | 1.10               |
| 27          | N-phenyl-1-naphthyl-amine.                                          | 2                                                    | Potassium (p-nonyl-phenoxide)                                                                                                                                                            | 0.065                                                | 0.01-K.....                                                                  | 140                       | 17.45                               | 0.65               |
| 28          | 5-ethyl-10,10-diphenyl-phenazasiline.                               | 2                                                    | None.....                                                                                                                                                                                |                                                      |                                                                              | 20                        | 190                                 | 20.7               |
|             | 5-ethyl-10,10-diphenyl-phenazasiline.                               | 2                                                    | Potassium (p-nonyl-phenoxide)                                                                                                                                                            | 0.065                                                | 0.01-K.....                                                                  | 40                        | 29                                  | 4.2                |
| 29          | N-ethylphenothiazine-P,P'-dioctyldiphenyl-amine.                    | 1<br>1                                               | None.....                                                                                                                                                                                |                                                      |                                                                              | 40                        | 37.7                                | 12.8               |
|             | N-ethylphenothiazine-P,P'-dioctyldiphenyl-amine.                    | 1<br>1                                               | Sodium stearate.....                                                                                                                                                                     | 0.27                                                 | 0.02-Na.....                                                                 | 20                        | 36.8                                | 8.4                |
| 30          | N-phenyl-1-naphthyl-amine.<br>P,P'-dioctyldiphenyl-amine.           | 1<br>1                                               | None.....                                                                                                                                                                                |                                                      |                                                                              | 20                        | 36.8                                | 8.4                |
|             | N-phenyl-1-naphthyl-amine.<br>P,P'-dioctyldiphenyl-amine.           | 1<br>1                                               | Sodium stearate.....                                                                                                                                                                     | 0.27                                                 | 0.02-Na.....                                                                 | 100                       | 22.8                                | 1.85               |
| 31          | N-phenyl-1-naphthylamine-P,P'-dioctyldiphenyl-amine.                | 1                                                    | Potassium salt of imide-amide reaction product of Acid No. 49 and derived from EDTA and C <sub>12</sub> -C <sub>15</sub> t-alkyl primary amine mixture reacted on 1:3 mole ratio basis.  | 0.25                                                 | 0.01-K.....                                                                  | 120                       | 26.6                                | 1.60               |

TABLE III—Continued

| Example No. | Arylamine Antioxidant Portion              |                                                      | Alkali Metal Salt Portion                                                                                                                                                               |                                                      |                                                                              | 425° F. AF Oxidation Test |                                     |          |
|-------------|--------------------------------------------|------------------------------------------------------|-----------------------------------------------------------------------------------------------------------------------------------------------------------------------------------------|------------------------------------------------------|------------------------------------------------------------------------------|---------------------------|-------------------------------------|----------|
|             | Component(s)                               | Concentration in percent by wt. of ester oil portion | Component(s)                                                                                                                                                                            | Concentration in percent by wt. of ester oil portion | Equivalent alkali metal concentration in percent by wt. of ester oil portion | Oxidation time in hours   | Viscosity in centistokes at 100° F. | Acid No. |
|             | N-phenyl-1-naphthylamine.<br>Diphenylamine | 1<br>1                                               | None                                                                                                                                                                                    |                                                      |                                                                              | 20                        | 42.6                                | 10.7     |
| 32          | N-phenyl-1-naphthylamine.<br>Diphenylamine | 1<br>1                                               | Potassium salt of imide-amide reaction product of Acid No. 49 and derived from EDTA and C <sub>12</sub> -C <sub>15</sub> t-alkyl primary amine mixture reacted on 1:3 mole ratio basis. | 0.50                                                 | 0.02-K                                                                       | 140                       | 16.3                                | 0.00     |
|             | N,N'-di(β-naphthyl)-p-phenylenediamine.    | 2                                                    | None                                                                                                                                                                                    |                                                      |                                                                              | 40                        | 40.1                                | 9.0      |
| 33          | N,N'-di(β-naphthyl)-p-phenylenediamine.    | 2                                                    | Potassium salt of imide-amide reaction product of Acid No. 49 and derived from EDTA and C <sub>12</sub> -C <sub>15</sub> t-alkyl primary amine mixture reacted on 1:3 mole ratio basis. | 0.25                                                 | 0.01-K                                                                       | 80                        | 20.8                                | 2.18     |
|             | Phenothiazine                              | 1                                                    | None                                                                                                                                                                                    |                                                      |                                                                              | 40                        | 26.9                                | 5.4      |
| 34          | Phenothiazine                              | 1                                                    | Potassium salt of imide-amide reaction product of Acid No. 49 and derived from EDTA and C <sub>12</sub> -C <sub>15</sub> t-alkyl primary amine mixture reacted on 1:3 mole ratio basis. | 0.25                                                 | 0.01-K                                                                       | 40                        | 18.7                                | 4.3      |

Thus, there are provided more, specific ester oil compositions useful as high temperature lubricants.

*Examples 35-41*

These examples illustrate specific embodiments of the ester oil lubricant of this invention, which embodiments involve other esters which are oils at 20-25° C. and which are used as base stocks for lubricants.

The esters called for by the formulations of each of these specific embodiments are indicated in the following Table IV. The arylamine antioxidant portion of each of the specific embodiments of Examples 35 and 36 consists essentially of N-phenyl-1-naphthylamine at a concentration of 0.5% by weight of the ester oil portion of these specific embodiments and 5-ethyl-10,10-diphenylphenazasiline at a concentration of 0.5% by weight of the ester oil portion of these specific embodiments. The arylamine

antioxidant portion of each of the specific embodiments of Examples 37-41 consists essentially of N-phenyl-1-naphthylamine at a concentration of 1% by weight of the ester oil portion of each of these specific embodiments and 5-ethyl-10,10-diphenylphenazasiline at a concentration of 1% by weight of the ester oil portion of each of these specific embodiments. The composition (components, concentrations and equivalent alkali metal concentrations) of the alkali metal salt portion of each specific embodiment is presented in Table IV.

These specific embodiments likewise are made by blending together the components at 50-90° C.

Table IV also contains typical data actually obtained in running the 425° F. AF Oxidation Test on samples of these specific embodiments and on the indicated ester oils containing only the corresponding arylamine antioxidant portions just described.

TABLE IV

| Example No. | Ester Oil Portion                                 | Alkali Metal Salt Portion                                                                                                                                                               |                                                      |                                                                              | 425° F. AF Oxidation Test |                                     |               |
|-------------|---------------------------------------------------|-----------------------------------------------------------------------------------------------------------------------------------------------------------------------------------------|------------------------------------------------------|------------------------------------------------------------------------------|---------------------------|-------------------------------------|---------------|
|             |                                                   | Component(s)                                                                                                                                                                            | Concentration in percent by wt. of ester oil portion | Equivalent alkali metal concentration in percent by wt. of ester oil portion | Oxidation time in hours   | Viscosity in centistokes at 100° F. | Acid No.      |
|             | 2-ethyl-2-isobutyl-1,3-propanediol dipelargonate. | None                                                                                                                                                                                    |                                                      |                                                                              | 0<br>20                   | 13.83<br>47.4                       | 0.02<br>10.60 |
| 35          | 2-ethyl-2-isobutyl-1,3-propanediol dipelargonate. | Sodium stearate                                                                                                                                                                         | 0.13                                                 | 0.01-Na                                                                      | 120                       | 17.9                                | 0.76          |
|             | Bis(2,2,4-trimethylpentyl)azelate.                | None                                                                                                                                                                                    |                                                      |                                                                              | 0<br>20                   | 13.82<br>47.0                       | 0.04<br>20.9  |
| 36          | Bis(2,2,4-trimethylpentyl)azelate.                | Potassium(p-nonylphenoxide)                                                                                                                                                             | 0.065                                                | 0.01-K                                                                       | 140                       | 17.2                                | 0.59          |
|             | Trimethylolpropanetriheptanoate.                  | None                                                                                                                                                                                    |                                                      |                                                                              | 0<br>20                   | 15.26<br>26.9                       | 0.04<br>4.19  |
| 37          | Trimethylolpropanetriheptanoate.                  | Potassium salt of imide-amide reaction product of Acid No. 49 and derived from EDTA and C <sub>12</sub> -C <sub>15</sub> t-alkyl primary amine mixture reacted on 1:3 mole ratio basis. | 0.25                                                 | 0.01-K                                                                       | 60                        | 16.4                                | 0.00          |
|             | Pentaerythritoltetrahexanoate                     | None                                                                                                                                                                                    |                                                      |                                                                              | 0<br>40                   | 28.26<br>83.8                       | 0.19<br>4.3   |

TABLE IV—Continued

| Example No. | Ester Oil Portion                                                                                                            | Alkali Metal Salt Portion                                                                                                                                                               |                                                      |                                                                              | 425° F. AF Oxidation Test |                                     |              |
|-------------|------------------------------------------------------------------------------------------------------------------------------|-----------------------------------------------------------------------------------------------------------------------------------------------------------------------------------------|------------------------------------------------------|------------------------------------------------------------------------------|---------------------------|-------------------------------------|--------------|
|             |                                                                                                                              | Component(s)                                                                                                                                                                            | Concentration in percent by wt. of ester oil portion | Equivalent alkali metal concentration in percent by wt. of ester oil portion | Oxidation time in hours   | Viscosity in centistokes at 100° F. | Acid No.     |
| 38          | Pentaerythritoltetrahexanoate                                                                                                | Potassium salt of imide-amide reaction product of Acid No. 49 and derived from EDTA and C <sub>12</sub> -C <sub>15</sub> t-alkyl primary amine mixture reacted on 1:3 mole ratio basis. | 0.25                                                 | 0.01-K                                                                       | 120                       | 35.4                                | 0.31         |
|             | 2,2,4-trimethyl-1,3-pentanediol dipelargonate.                                                                               | None                                                                                                                                                                                    |                                                      |                                                                              | 0<br>20                   | 12.31<br>26.8                       | 0.07<br>7.5  |
| 39          | 2,2,4-trimethyl-1,3-pentanediol dipelargonate.                                                                               | Potassium salt of imide-amide reaction product of Acid No. 49 and derived from EDTA and C <sub>12</sub> -C <sub>15</sub> t-alkyl primary amine mixture reacted on 1:3 mole ratio basis. | 0.25                                                 | 0.01-K                                                                       | 120                       | 17.5                                | 0.45         |
|             | Bis(2-ethylhexyl) sebacate                                                                                                   | None                                                                                                                                                                                    |                                                      |                                                                              | 0<br>60                   | 13.0<br>41.0                        | 0.05<br>22.7 |
| 40          | Bis(2-ethylhexyl) sebacate                                                                                                   | Potassium salt of imide-amide reaction product of Acid No. 49 and derived from EDTA and C <sub>12</sub> -C <sub>15</sub> t-alkyl primary amine mixture reacted on 1:3 mole ratio basis. | 0.25                                                 | 0.01-K                                                                       | 120                       | 16.9                                | 0.85         |
|             | Polyester of neopentyl glycol and sebadic acid, and terminated with 2-ethylhexanol, all reacted on a 2:1:2 mole ratio basis. | None                                                                                                                                                                                    |                                                      |                                                                              | 0<br>40                   | 1,585<br>7,652                      | 1.06<br>4.80 |
| 41          | Polyester of neopentyl glycol and sebadic acid, and terminated with 2-ethylhexanol, all reacted on a 2:1:2 mole ratio basis. | Potassium salt of imide-amide reaction product of Acid No. 49 and derived from EDTA and C <sub>12</sub> -C <sub>15</sub> t-alkyl primary amine mixture reacted on 1:3 mole ratio basis. | 0.25                                                 | 0.01-K                                                                       | 40                        | 4,469                               | 2.64         |

Thus, there are provided a number of embodiments of the ester oil lubricant composition of this invention, which are based on various ester oils.

#### Examples 42-53

These examples illustrate more, specific embodiments of the ester oil compositions of this invention.

The ester oils in the formulations of each of these specific embodiments are identified in the following Table V. The composition of the arylamine antioxidant portion and the composition of the alkali metal salt portion are also set forth in Table V.

These specific embodiments are made by admixing the components at 50-90° C.

Table V also presents typical data actually obtained in testing for oxidative stability samples of these specific embodiments. The test employed is referred to herein as the 500° F. oxidation test. In this test 36 liters of air per hour are passed through a 25 milliliter sample of the oil composition under test, which sample contains a 1 inch length of  $\frac{1}{16}$  diameter, freshly polished, iron wire. While the air is passed through the sample, the temperature of the sample is established and maintained at about 500° F.

TABLE V

| Ex. No. | Ester Oil Portion                                    | Arylamine Antioxidant Portion                                              |            | Alkali Metal Salt Portion                                                                                                                                                               |            |                                      | 500° F. Oxidation Test Results                                          |                                       |                                                     |              |
|---------|------------------------------------------------------|----------------------------------------------------------------------------|------------|-----------------------------------------------------------------------------------------------------------------------------------------------------------------------------------------|------------|--------------------------------------|-------------------------------------------------------------------------|---------------------------------------|-----------------------------------------------------|--------------|
|         |                                                      | Components                                                                 | Components | Concen-<br>tra-<br>tion <sup>1</sup>                                                                                                                                                    | Components | Concen-<br>tra-<br>tion <sup>1</sup> | Equiv-<br>alent alkali<br>metal<br>concen-<br>tra-<br>tion <sup>1</sup> | Oxida-<br>tion<br>time<br>in<br>hours | Viscos-<br>ity in<br>centi-<br>stokes at<br>100° F. | Acid No.     |
|         | Pentaerythritol tetra (50/50 octanoate/pelargonate). | None                                                                       |            |                                                                                                                                                                                         | None       |                                      |                                                                         | 0<br>20                               | 34.01<br>(2)                                        | 0.00         |
|         | Pentaerythritol tetra (50/50 octanoate/pelargonate). | N-(p-dodecylphenyl)-2-naphthylamine. 5-Ethyl-10,10-diphenyl-phenazasiline. | 3.56<br>1  | None                                                                                                                                                                                    |            |                                      |                                                                         | 0<br>20                               | 38.01<br>8,000                                      | 0.00<br>16.2 |
| 42      | Pentaerythritol tetra (50/50 octanoate/pelargonate). | N-(p-dodecylphenyl)-2-naphthylamine. 5-Ethyl-10,10-diphenyl-phenazasiline. | 3.56<br>1  | Potassium salt of imide-amide reaction product of Acid No. 49 and derived from EDTA and C <sub>12</sub> -C <sub>15</sub> t-alkyl primary amine mixture reacted on 1:3 mole ratio basis. | 2.5        | 0.01-K                               |                                                                         | 80                                    | 69.5                                                | 0.13         |
| 43      | Pentaerythritol tetra (50/50 octanoate/pelargonate). | N-phenyl-1-naphthylamine. 5-ethyl-10,10-diphenyl-phenazasiline.            | 2<br>1     | Potassium salt of imide-amide reaction product of Acid No. 49 and derived from EDTA and C <sub>12</sub> -C <sub>15</sub> t-alkyl primary amine mixture reacted on 1:3 mole ratio basis. | 2.5        | 0.02-K                               |                                                                         | 0<br>20                               | 35.0<br>63.1                                        | 0.04<br>1.2  |

See footnotes at end of table.

TABLE V—Continued

| Ex. No. | Ester Oil Portion                                             | Arylamine Antioxidant Portion                                                |                            | Alkali Metal Salt Portion                                                                                                                                                               |                            |                                                    | 500° F. Oxidation Test Results |                                     |                    |
|---------|---------------------------------------------------------------|------------------------------------------------------------------------------|----------------------------|-----------------------------------------------------------------------------------------------------------------------------------------------------------------------------------------|----------------------------|----------------------------------------------------|--------------------------------|-------------------------------------|--------------------|
|         | Components                                                    | Components                                                                   | Concentration <sup>1</sup> | Components                                                                                                                                                                              | Concentration <sup>1</sup> | Equivalent alkali metal concentration <sup>1</sup> | Oxidation time in hours        | Viscosity in centistokes at 100° F. | Acid No.           |
| 44      | Pentaerythritol tetra (50/50 octanoate/pelargonate).          | N-phenyl-1-naphthylamine-5-ethyl-10,10-diphenylphenazasiline.                | 2 1                        | Potassium (p-nonylphenoxide).                                                                                                                                                           | 0.13                       | 0.02—K---                                          | 0 20                           | 35.0 54.1                           | 0.01 0.76          |
| 45      | Pentaerythritol tetra (50/50 octanoate/pelargonate).          | p-Octyldiphenylamine-5-ethyl-10,10-diphenylphenazasiline.                    | 2.60 1                     | Potassium salt of imide-amide reaction product of Acid No. 49 and derived from EDTA and C <sub>12</sub> -C <sub>15</sub> t-alkyl primary amine mixture reacted on 1:3 mole ratio basis. | 0.5                        | 0.02—K---                                          | 20                             | 54.1                                | 0.73               |
| 46      | Pentaerythritol tetra (50/50 octanoate/pelargonate).          | N-(p-dodecylphenyl)-1-naphthylamine-5-ethyl-10,10-diphenylphenazasiline.     | 3.56 1                     | Potassium salt of imide-amide reaction product of Acid No. 49 and derived from EDTA and C <sub>12</sub> -C <sub>15</sub> t-alkyl primary amine mixture reacted on 1:3 mole ratio basis. | 0.5                        | 0.02—K---                                          | 20                             | 50.71                               | 0.85               |
| 47      | Pentaerythritol tetra (50/50 octanoate/pelargonate).          | Di-2-naphthylamine-5-ethyl-10,10-diphenylphenazasiline.                      | 2.47 1                     | Potassium salt of imide-amide reaction product of Acid No. 49 and derived from EDTA and C <sub>12</sub> -C <sub>15</sub> t-alkyl primary amine mixture reacted on 1:3 mole ratio basis. | 0.5                        | 0.02—K---                                          | 20                             | 45.1                                | 0.28               |
| 48      | Pentaerythritol tetra (50/50 octanoate/pelargonate).          | N-butyldiphenylamine-5-ethyl-10,10-diphenylphenazasiline.                    | 2 1                        | Potassium salt of imide-amide reaction product of Acid No. 49 and derived from EDTA and C <sub>12</sub> -C <sub>15</sub> t-alkyl primary amine mixture reacted on 1:3 mole ratio basis. | 0.5                        | 0.02—K---                                          | 20                             | 61.0                                | 0.—<br>95          |
| 49      | Pentaerythritol tetra (50/50 octanoate/pelargonate).          | Dodecyl ester of 2-anilino-benzoic acid-5-ethyl-10,10-diphenylphenazasiline. | 3.48 1                     | Potassium salt of imide-amide reaction product of Acid No. 49 and derived from EDTA and C <sub>12</sub> -C <sub>15</sub> t-alkyl primary amine mixture reacted on 1:3 mole ratio basis. | 0.5                        | 0.02—K---                                          | 20                             | 63.7                                | 0.—<br>85          |
| 50      | Pentaerythritol tetra (50/50 octanoate/pelargonate).          | N-(p-dodecylphenyl)-2-naphthylamine-5-ethyl-10,10-diphenylphenazasiline.     | 3.56 1                     | Potassium salt of imide-amide reaction product of Acid No. 49 and derived from EDTA and C <sub>12</sub> -C <sub>15</sub> t-alkyl primary amine mixture reacted on 1:3 mole ratio basis. | 5                          | 0.20—K---                                          | 0 100                          | 45.16 81.8                          | 0.—<br>87<br>0. 45 |
| 51      | Pentaerythritol tetra (50/50 octanoate/pelargonate).          | N-(p-dodecylphenyl)-2-naphthylamine.                                         | 3.56                       | Potassium salt of imide-amide reaction product of Acid No. 49 and derived from EDTA and C <sub>12</sub> -C <sub>15</sub> t-alkyl primary amine mixture reacted on 1:3 mole ratio basis. | 2.5                        | 0.10—K---                                          | 0 60                           | 40.20 62.6                          | 0.—<br>43<br>0. 71 |
| 52      | 2-butyl-2-ethyl-1,3-propanediol dilaurate.                    | N-(p-dodecylphenyl)-2-naphthylamine-5-ethyl-10,10-diphenylphenazasiline.     | 3.56 1                     | Potassium salt of imide-amide reaction product of Acid No. 49 and derived from EDTA and C <sub>12</sub> -C <sub>15</sub> t-alkyl primary amine mixture reacted on 1:3 mole ratio basis. | 0.50                       | 0.02—K---                                          | 0 20                           | 27.66 35.3                          | 0.—<br>05<br>1. 2  |
| 53      | 2,4-dimethyl-2,4,di-propyl-1,3-cyclobutanediol diundecanoate. | N-(p-dodecylphenyl)-2-naphthylamine-5-ethyl-10,10-diphenylphenazasiline.     | 3.56 1                     | Potassium salt of imide-amide reaction product of Acid No. 49 and derived from EDTA and C <sub>12</sub> -C <sub>15</sub> t-alkyl primary amine mixture reacted on 1:3 mole ratio basis. | 2.5                        | 0.10—K---                                          | 0 20                           | 39.10 52.9                          | 0.—<br>41<br>1. 2  |

<sup>1</sup> In percent by weight of ester oil portion. <sup>2</sup> Thick grease.

## Examples 54-60

These examples illustrate still more embodiments of the ester oil composition of this invention.

The ester oil portion in each of these specific embodiments consists essentially of 2-butyl-2-ethyl-1,3-propanediol dipelargonate. The arylamine antioxidant portion in each of these specific embodiments consists essentially of N-phenyl-1-naphthylamine at a concentration of 1% of the weight of the ester oil portion and 5-ethyl-10,10-diphenylphenazasiline at a concentration of 1% of the weight of the ester oil portion. The composition of the alkali metal salt portion is given in the following Table VI.

These specific embodiments are made by thoroughly blending together the components at 50-90° C.

Samples of these specific embodiments as well as of the ester oil portion alone, with an arylamine antioxidant portion only and with an alkali metal salt portion only were actually prepared and tested for oxidative stability

70 at 425° F. The test employed is a modified 425° F. AF Oxidation Test. The procedure and conditions are the same as described in conjunction with Examples 1-17, except a stainless steel coupon is used in place of the titanium coupon. The test results are summarized in Table VI.

75

TABLE VI

| Example No. | Alkali Metal Salt Portion                                                                                                                                                                                                                                                                                                           |                                                              |                                                                              | Modified 425° F. AF Oxidation Test Results |                                      |                       |
|-------------|-------------------------------------------------------------------------------------------------------------------------------------------------------------------------------------------------------------------------------------------------------------------------------------------------------------------------------------|--------------------------------------------------------------|------------------------------------------------------------------------------|--------------------------------------------|--------------------------------------|-----------------------|
|             | Components                                                                                                                                                                                                                                                                                                                          | Concentration of salt in percent by wt. of ester oil portion | Equivalent alkali metal concentration in percent by wt. of ester oil portion | Oxidation time in hours                    | Viscosity in centi-stokes at 100° F. | Acid No.              |
| 54          | Potassium salt of 1-naphthol                                                                                                                                                                                                                                                                                                        | 0.046                                                        | 0.01-K                                                                       | 0<br>120                                   | 14.45<br>15.97                       | 0.02<br>0.38          |
| 55          | Potassium salt of 1-hydroxyanthraquinone                                                                                                                                                                                                                                                                                            | 0.067                                                        | 0.01-K                                                                       | 0<br>40                                    | 14.74<br>17.74                       | 0.03<br>2.50          |
| 56          | Potassium salt of 1-phenylazo-2-naphthol                                                                                                                                                                                                                                                                                            | 0.073                                                        | 0.01-K                                                                       | 0<br>120                                   | 15.44<br>18.69                       | 0.01<br>0.70          |
| 57          | Potassium salt of neotridecanoic acid                                                                                                                                                                                                                                                                                               | 0.065                                                        | 0.01-K                                                                       | 0<br>120                                   | 14.90<br>17.62                       | 0.02<br>0.72          |
| 58          | Sodium salt of neotridecanoic acid                                                                                                                                                                                                                                                                                                  | 0.061                                                        | 0.006-Na                                                                     | 0<br>120                                   | 14.76<br>19.34                       | 0.03<br>1.54          |
| 59          | Dipotassium salt of acid terminated polyester of pimelic acid and 1,4-cyclohexanedimethanol reacted on a 1:1 mole ratio basis.                                                                                                                                                                                                      | 0.26                                                         | 0.01-K                                                                       | 0<br>120                                   | 14.36<br>22.67                       | 0.01<br>2.00          |
| 60          | Potassium salt of naphthenic acid product of average molecular weight of 310 and Acid No. of 169. (Sunaptic Acid A).                                                                                                                                                                                                                | 0.088                                                        | 0.01-K                                                                       | 0<br>120                                   | 15.05<br>18.35                       | 0.01<br>0.88          |
|             | Ester oil without any arylamine antioxidants but with potassium salt of naphthenic acid product of average molecular weight of 310 and Acid No. of 169 (Sunaptic Acid A), the salt being present at a concentration of 0.088% by weight of the ester oil and equivalent to K concentration of 0.01% of the weight of the ester oil. |                                                              |                                                                              | 0<br>120                                   | 13.89<br>71.77                       | 0.02<br>12.56         |
|             | Ester oil without any arylamine antioxidants and without any alkali metal salts                                                                                                                                                                                                                                                     |                                                              |                                                                              | 0<br>20                                    | 14.32<br>229                         | 0.0<br>18.7           |
|             | Ester oil with arylamine antioxidants but without any alkali metal salts                                                                                                                                                                                                                                                            |                                                              |                                                                              | 0<br>20<br>40                              | 15.09<br>43.8<br>152                 | 0.02<br>9.80<br>11.69 |

*Examples 61-69*

These examples illustrate more embodiments of the ester oil composition of this invention.

2-butyl-2-ethyl-1,3-propanediol dipelargonate is the ester oil portion of these embodiments. The compositions and concentrations of the arylamine antioxidant portion and the alkali metal salt portion of these embodiments are given in the following Table VII.

The octylated styrenated diphenylamine product called for by some of the formulations involved in these specific embodiments is a normally liquid, oily product consisting essentially of (1) p,p'-di-t-octyldiphenylamine, (2) p,p'-di- $\alpha$ -phenethyldiphenylamine, (3) p-t-octyl-p'- $\alpha$ -phenethyldiphenylamine, (4) p-mono-t-octyldiphenylamine and (5) p-mono- $\alpha$ -phenethyldiphenylamine in the ratio of 50-70% by weight of (1), (2), and (3) to 30-50% by weight of (4) and (5), said product resulting from the reaction of 1.3 to 2.0 chemical equivalents of a hydrocarbon mixture containing diisobutylene and styrene in the ratio of 2-5 parts by weight of diisobutylene to 1 part by weight

of styrene, with one chemical equivalent of diphenylamine with the aid of a Friedel-Crafts condensation catalyst such as aluminum chloride, at a temperature of 150-200° C. This product and its synthesis is described in the U.S. patent, No. 2,530,769, to Hollis. It is marketed as Goodrite Staylite.

The octylated diphenylamine product called for in these embodiments is a mixture consisting essentially of diphenylamines substituted by octyl groups. The mixture is derived from diphenylamine. The product is available commercially as Vanlube 60.

The specific embodiments involved in these examples are made by thoroughly blending together the components at 50-90° C.

Samples of these specific embodiments as well as of the ester oil portion alone, with an arylamine antioxidant portion alone were actually prepared and tested for oxidation stability by the modified 425° F. AF Oxidation Test described in conjunction with Examples 54-60. The test results are set forth in Table VII.

TABLE VII

| Example No. | Arylamine Antioxidant Portion               |                                                      | Alkali Metal Salt Portion                                                                                                                                                               |                                                      |                                                                              | Modified 425° F. AF Oxidation Test |                                      |              |
|-------------|---------------------------------------------|------------------------------------------------------|-----------------------------------------------------------------------------------------------------------------------------------------------------------------------------------------|------------------------------------------------------|------------------------------------------------------------------------------|------------------------------------|--------------------------------------|--------------|
|             | Component(s)                                | Concentration in percent by wt. of ester oil portion | Component(s)                                                                                                                                                                            | Concentration in percent by wt. of ester oil portion | Equivalent alkali metal concentration in percent by wt. of ester oil portion | Oxidation time in hours            | Viscosity in centi-stokes at 100° F. | Acid No.     |
|             | Octylated styrenated diphenylamine product. | 1                                                    | None                                                                                                                                                                                    |                                                      |                                                                              | 0<br>20                            | 14.24<br>81.3                        | 0.03<br>9.66 |
| 61          | Octylated styrenated diphenylamine product. | 1                                                    | Potassium salt of imide-amide reaction product of Acid No. 49 and derived from EDTA and C <sub>12</sub> -C <sub>15</sub> t-alkyl primary amine mixture reacted on 1:3 mole ratio basis. | 0.5                                                  | 0.02-K                                                                       | 0<br>140                           | 14.65<br>18.71                       | 0.03<br>0.39 |

TABLE VII—Continued

| Example No. | Arylamine Antioxidant Portion                                  |                                                      | Alkali Metal Salt Portion                                                                                                                                                               |                                                      |                                                                              | Modified 425° F. AF Oxidation Test |                                     |              |
|-------------|----------------------------------------------------------------|------------------------------------------------------|-----------------------------------------------------------------------------------------------------------------------------------------------------------------------------------------|------------------------------------------------------|------------------------------------------------------------------------------|------------------------------------|-------------------------------------|--------------|
|             | Component(s)                                                   | Concentration in percent by wt. of ester oil portion | Component(s)                                                                                                                                                                            | Concentration in percent by wt. of ester oil portion | Equivalent alkali metal concentration in percent by wt. of ester oil portion | Oxidation time in hours            | Viscosity in centistokes at 100° F. | Acid No.     |
| 62-----     | Octylated styrenated diphenylamine product.                    | 2                                                    | Potassium salt of naphthenic acid product of average molecular weight of 310 and Acid No. of 169. (Sunaptic Acid A).                                                                    | 0.18                                                 | 0.02—K-----                                                                  | 0<br>80                            | 16.43<br>21.60                      | 0.05<br>0.77 |
|             | Octylated diphenylamine product.                               |                                                      | None-----                                                                                                                                                                               |                                                      |                                                                              |                                    |                                     |              |
| 63-----     | Octylated diphenylamine product.                               | 1                                                    | Potassium salt of imide-amide reaction product of Acid No. 49 and derived from EDTA and C <sub>12</sub> —C <sub>15</sub> t-alkyl primary amine mixture reacted on 1:3 mole ratio basis. | 0.5                                                  | 0.02—K-----                                                                  | 0<br>140                           | 14.35<br>18.58                      | 0.02<br>0.29 |
|             | p,p'-Diocetyl diphenylamine.                                   |                                                      | Potassium salt of imide-amide reaction product of Acid No. 49 and derived from EDTA and C <sub>12</sub> —C <sub>15</sub> t-alkyl primary amine mixture reacted on 1:3 mole ratio basis. |                                                      |                                                                              |                                    |                                     |              |
| 64-----     | N-(p-dodecylphenyl)-2-naphthylamine.                           | 3.6                                                  | Potassium salt of imide-amide reaction product of Acid No. 49 and derived from EDTA and C <sub>12</sub> —C <sub>15</sub> t-alkyl primary amine mixture reacted on 1:3 mole ratio basis. | 0.25                                                 | 0.01—K-----                                                                  | 0<br>80                            | 16.12<br>24.83                      | 0.01<br>0.30 |
|             | Octylated styrenated diphenylamine product.                    |                                                      | None-----                                                                                                                                                                               |                                                      |                                                                              |                                    |                                     |              |
| 65-----     | Octylated styrenated diphenylamine product.                    | 0.4                                                  | Potassium salt of imide-amide reaction product of Acid No. 49 and derived from EDTA and C <sub>12</sub> —C <sub>15</sub> t-alkyl primary amine mixture reacted on 1:3 mole ratio basis. | 0.25                                                 | 0.01—K-----                                                                  | 0<br>80                            | 13.89<br>46.88                      | 0.01<br>0.35 |
|             | N-phenyl-1-naphthylamine, 5-ethyl-10,10-diphenylphenazasiline. |                                                      | None-----                                                                                                                                                                               |                                                      |                                                                              |                                    |                                     |              |
| 66-----     | N-phenyl-1-naphthylamine, 5-ethyl-10,10-diphenylphenazasiline. | 1                                                    | Sodium stearate-----                                                                                                                                                                    | 0.064                                                | 0.005—Na-----                                                                | 0<br>120                           | 14.55<br>18.35                      | 0.03<br>1.11 |
|             | N-phenyl-1-naphthylamine, 5-ethyl-10,10-diphenylphenazasiline. |                                                      | Potassium salt of naphthenic acid product of average molecular weight of 310 and Acid No. of 169. (Sunaptic Acid A).                                                                    |                                                      |                                                                              |                                    |                                     |              |
| 67-----     | N-phenyl-1-naphthylamine.                                      | 1                                                    | None-----                                                                                                                                                                               | 5.6                                                  | 0.63—K-----                                                                  | 0<br>100                           | 14.88<br>17.45                      | 0.03<br>0.28 |
|             | 5-ethyl-10,10-diphenylphenazasiline.                           |                                                      | Sodium stearate-----                                                                                                                                                                    |                                                      |                                                                              |                                    |                                     |              |
| 68-----     | N-phenyl-1-naphthylamine.                                      | 1                                                    | Potassium salt of naphthenic acid product of average molecular weight of 310 and Acid No. of 169. (Sunaptic Acid A).                                                                    | 1.0                                                  | 0.11—K-----                                                                  | 0<br>120                           | 15.44<br>17.83                      | 0.01<br>3.49 |
|             | 5-ethyl-10,10-diphenylphenazasiline.                           |                                                      | None-----                                                                                                                                                                               |                                                      |                                                                              |                                    |                                     |              |
| 69-----     | N-phenyl-1-naphthylamine.                                      | 5                                                    | Potassium salt of naphthenic acid product of average molecular weight of 310 and Acid No. of 169. (Sunaptic Acid A).                                                                    |                                                      |                                                                              |                                    |                                     |              |
|             | N-phenyl-1-naphthylamine.                                      |                                                      | None-----                                                                                                                                                                               |                                                      |                                                                              |                                    |                                     |              |

## Examples 70-76

These examples illustrate additional specific embodiments of the ester oil composition of this invention.

The ester oil portion, the arylamine antioxidant portion and the alkali metal salt portion of these specific embodiments are given in the following Table VIII. The octylated styrenated diphenylamine product is described in conjunction with Examples 61-69.

These specific embodiments are made by thoroughly mixing together at 50-90° C. the components thereof.

Table VIII also contains the results obtained in actually

65 testing samples for oxidative stability samples of these embodiments as well as of the ester oil portion of these embodiments the ester oil portion plus one or the other, as indicated in Table VIII, of a specific arylamine antioxidant portion and of a specific alkali metal salt portion 70 involved in these embodiments. The test employed here is a modification of the 425° F. AF Oxidation Test in that instead of a copper coupon a stainless steel coupon is employed and the temperature of the sample is established and maintained at 500° F. This test is hereinafter referred to as the 500° F. AF Oxidation Test.

TABLE VIII

| Ex. No. | Ester Oil Portion                                                 | Arylamine Antioxidant Portion                                        |                                      | Alkali Metal Salt Portion                                                                                                                                                               |                                      |                                                                           | 500° F. AF Oxidation Test Results  |                                                     |              |
|---------|-------------------------------------------------------------------|----------------------------------------------------------------------|--------------------------------------|-----------------------------------------------------------------------------------------------------------------------------------------------------------------------------------------|--------------------------------------|---------------------------------------------------------------------------|------------------------------------|-----------------------------------------------------|--------------|
|         | Components                                                        | Components                                                           | Concen-<br>tra-<br>tion <sup>1</sup> | Components                                                                                                                                                                              | Concen-<br>tra-<br>tion <sup>1</sup> | Equiva-<br>lent alkali<br>metal con-<br>cen-<br>tra-<br>tion <sup>1</sup> | Oxida-<br>tion<br>time<br>in hours | Viscos-<br>ity in<br>centi-<br>stokes at<br>100° F. | Acid<br>No.  |
|         | Pentaerythritol tetra-(75/25 pelargonate/2-ethyl hexanoate).      | None.....                                                            |                                      | None.....                                                                                                                                                                               |                                      |                                                                           | 0<br>20                            | 37.90<br>>2000                                      | 0.04<br>7.10 |
|         | Pentaerythritol tetra-(75/25 pelargonate/2-ethyl hexanoate).      | p,p'-Diocetylphenylamine                                             | 3                                    | None.....                                                                                                                                                                               |                                      |                                                                           | 0<br>20                            | 39.27<br>300                                        | 0.06<br>5.83 |
|         | Pentaerythritol tetra-(75/25 pelargonate/2-ethyl hexanoate).      | None.....                                                            |                                      | Potassium salt of naphthenic acid product of average molecular wt. of 310 and Acid No. of 169 (Sunaptic Acid A).                                                                        | 0.9<br>0.9                           | 0.1-K....                                                                 | 0<br>20                            | 41.0<br>1900                                        | 0.30<br>6.22 |
| 70      | Pentaerythritol tetra-(75/25 pelargonate/2-ethyl hexanoate).      | p,p'-Diocetylphenylamine                                             | 3                                    | Potassium salt of naphthenic acid product of average molecular wt. of 310 and Acid No. of 169 (Sunaptic Acid A).                                                                        | 0.9                                  | 0.1-K....                                                                 | 0<br>140                           | 41.54<br>68.94                                      | 0.33<br>0.50 |
| 71      | Pentaerythritol tetra-(75/25 pelargonate/2-ethyl hexanoate).      | p,p'-Diocetylphenylamine-Octylated styrenated diphenylamine product. | 2.5<br>0.5                           | Potassium salt of naphthenic acid product of average molecular wt. of 310 and Acid No. of 169 (Sunaptic Acid A).                                                                        | 0.9                                  | 0.1-K....                                                                 | 0<br>140                           | 39.79<br>65.77                                      | 0.31<br>0.27 |
| 72      | Pentaerythritol tetra-(75/25 pelargonate/2-ethyl hexanoate).      | p,p'-Diocetylphenylamine-5-ethyl-10,10-diphenylphenazasiline.        | 2.5<br>0.5                           | Potassium salt of naphthenic acid product of average molecular wt. of 310 and Acid No. of 169 (Sunaptic Acid A).                                                                        | 0.9                                  | 0.1-K....                                                                 | 0<br>140                           | 40.46<br>63.93                                      | 0.31<br>0.44 |
| 73      | Pentaerythritol tetra-(75/25 pelargonate/2-ethylhexanoate).       | N-ethyl-p,p'-diocetylphenylamine.                                    | 2                                    | Potassium salt of imide-amide reaction product of Acid No. 49 and derived from EDTA and C <sub>12</sub> -C <sub>15</sub> t-alkyl primary amine mixture reacted on 1:3 mole ratio basis. | 1                                    | 0.04-K....                                                                | 0<br>40                            | 88.97<br>85.89                                      | 0.05<br>1.21 |
| 74      | Pentaerythritol tetra-(50/50 octanoate/pelargonate).              | Octylated styrenated diphenylamine product.                          | 5                                    | Potassium salt of naphthenic acid product of average molecular wt. of 310 and Acid No. of 169 (Sunaptic Acid A).                                                                        | 2.5                                  | 0.28-K....                                                                | 0<br>80                            | 41.60<br>67.98                                      | 0.05<br>0.54 |
| 75      | Pentaerythritol tetra-(60/50 pelargonate/2,2-dimethyl octanoate). | p,p'-Diocetylphenylamine                                             | 3                                    | Potassium salt of naphthenic acid product of average molecular wt. of 310 and Acid No. of 169 (Sunaptic Acid A).                                                                        | 0.9                                  | 0.01-K....                                                                | 0<br>120                           | 48.77<br>79.14                                      | 0.06<br>0.35 |
| 76      | Trimethylolpropane tripelargonate.                                | p,p'-Diocetylphenylamine                                             | 3                                    | Potassium salt of naphthenic acid product of average molecular wt. of 310 and Acid No. of 169 (Sunaptic Acid A).                                                                        | 0.44                                 | 0.05-K....                                                                | 0<br>60                            | 31.41<br>54.32                                      | 0.15<br>0.47 |

<sup>1</sup> In percent by weight of ester oil portion.

Thus, this invention provides an ester oil, lubricant composition having oxidative stability at temperatures over 300° F. and as high as 500° F.

From test data presented in the foregoing tables it is evident that not only does the arylamine antioxidant portion of the composition have antioxidant activity, but the alkali metal salt portion also has antioxidant activity. Moreover, the data suggest that the arylamine antioxidant portion and alkali metal salt portion of the composition of this invention function synergistically, that is to say, the antioxidant activity of the combination of the arylamine antioxidant portion and alkali metal salt portion is substantially greater than the mere addition of the antioxidant activity of the arylamine antioxidant portions alone and the antioxidant activity of the alkali metal salt portion alone. Further evidence of this synergistic effect is presented in connection with the following examples.

60

#### Examples 77-78

These examples illustrate two more, specific embodiments of the lubricant oil composition of this invention.

Table IX sets forth the ester oil portion, the arylamine antioxidant portion and the alkali metal salt portion of these specific embodiments. The octylated styrenated diphenylamine product called for in Table IX is described in conjunction with Examples 61-69.

These specific embodiments are made by admixing the components at 50-90° C.

70 Table IX also sets forth typical data obtained in actually subjecting to an oxidative stability test samples of these specific embodiments and of other compositions formulated as indicated in the table. The oxidative stability test employed in the Modified 425° F. AF Oxidation Test.

75

TABLE IX

| Ex. No. | Ester Oil Portion                              | Arylamine Antioxidant Portion                                 |                            |                                                                                                                                                                                         | Alkali Metal Salt Portion  |                                                    |                         | Modified 500° F. AF Oxidation Test Results |                      |  |
|---------|------------------------------------------------|---------------------------------------------------------------|----------------------------|-----------------------------------------------------------------------------------------------------------------------------------------------------------------------------------------|----------------------------|----------------------------------------------------|-------------------------|--------------------------------------------|----------------------|--|
|         | Components                                     | Components                                                    | Concentration <sup>1</sup> | Components                                                                                                                                                                              | Concentration <sup>1</sup> | Equivalent alkali metal concentration <sup>1</sup> | Oxidation time in hours | Viscosity in centistokes at 100° F.        | Acid No.             |  |
| 76      | 2-butyl-2-ethyl-1,3-propanediol dipelargonate. | Octylated styrenated diphenylamine product.                   | 1.5                        | None.....                                                                                                                                                                               |                            |                                                    | 0<br>20                 | 14.46<br>71.68                             | 0.01<br>10.96        |  |
|         | 2-butyl-2-ethyl-1,3-propanediol dipelargonate. | None.....                                                     |                            | Potassium salt of imide-amide reaction product of Acid No. 49 and derived from EDTA and C <sub>12</sub> -C <sub>15</sub> t-alkyl primary amine mixture reacted on 1:3 mole ratio basis. | 1.5                        | 0.06-K.....                                        | 0<br>20                 | 14.60<br>26.39                             | 0.30<br>3.25         |  |
| 77      | 2-butyl-2-ethyl-1,3-propanediol dipelargonate. | Octylated styrenated diphenylamine product.                   | 1.0                        | Potassium salt of imide-amide reaction product of Acid No. 49 and derived from EDTA and C <sub>12</sub> -C <sub>15</sub> t-alkyl primary amine mixture reacted on 1:3 mole ratio basis. | 0.5                        | 0.02-K.....                                        | 0<br>20<br>120          | 14.65<br>15.32<br>18.09                    | 0.03<br>0.54<br>0.23 |  |
| 78      | Trimethylolpropane triheptanoate.              | N-phenyl-1-naphthylamine-5-ethyl-10,10-diphenylphenazasiline. | 1.03<br>1.03               | None.....                                                                                                                                                                               |                            |                                                    | 0<br>40                 | 15.48<br>41.52                             | 0.02<br>7.66         |  |
|         | Trimethylolpropane triheptanoate.              | None.....                                                     |                            | Sodium salt of neotri-decanoic acid.                                                                                                                                                    | 2.06                       | 0.2-Na.....                                        | 0<br>40                 | 15.48<br>19.00                             | 0.04<br>0.70         |  |
| 78      | Trimethylolpropane triheptanoate.              | N-phenyl-1-naphthylamine-5-ethyl-10,10-diphenylphenazasiline. | 1.0<br>1.0                 | Sodium salt of neotri-decanoic acid.                                                                                                                                                    | 0.06                       | 0.006-Na.....                                      | 0<br>40                 | 15.73<br>17.07                             | 0.02<br>0.97         |  |

<sup>1</sup> In percent by weight of ester oil portion.

Not only do alkali metal salts of this invention activate arylamine antioxidants at temperatures of 425-500° F., but they also appear to activate the activity of arylamine antioxidants at lower temperatures. This is demonstrated by some actual test data obtained in running a variation of the well known 347° F. oxidation test described in Method 5308.4, of Federal Test Method Standard No. 791, which test is employed to evaluate jet lubes for Military Specification 7808D. In this variation, a 25 milliliter sample of the lubricant under test is heated in a 25 millimeter x 350 millimeter Pyrex tube topped with a water condenser. The temperature of the lubricant sample is established and maintained at 347° F. while 1.25 liters of air per hour are blown through the sample. Metal washers (3/4 inch diameter) of iron, copper, aluminum, magnesium and silver are disposed in the sample on the air delivery tube. Periodically, the acid number of the sample is determined. When the acid number has increased by 2.0, the period of time required to reach this condition is determined. This is referred to as the induction period or "stable life" of the lubricant. When this test was run on a sample of 2 - butyl-2-ethyl-1,3-propanediol dipelargonate containing N - phenyl-1-naphthylamine at a concentration of 1% by weight of the ester, the induction period was 265 hours. When the test was run on another sample of the 2-butyl-2-ethyl-1,3-propanediol dipelargonate containing not only N-phenyl-1-naphthylamine at a concentration of 1% by weight of the ester, but also the potassium salt of an imide-amide reaction product of Acid No. 49 and derived from EDTA

and a C<sub>12</sub>-C<sub>15</sub> t-alkyl primary amine mixture reacted on a 1:3 mole ratio basis with the salt being at a concentration of 0.25% by weight of the ester (equivalent to a potassium concentration of 0.01% by weight of the ester), the induction period was 381 hours.

The activation of arylamine antioxidants in synthetic ester oils at temperatures above 300° F. does not appear to be effected by other metal salts. This is demonstrated by the data presented relative to the following examples.

#### Examples 79-80

These examples illustrate still more specific embodiments of the lubricant oil composition of this invention. The ester oil portion of these examples consists essentially of 2-butyl-2-ethyl-1,3-propanediol dipelargonate. The arylamine antioxidant portion consists essentially of N-phenyl-1-naphthylamine at a concentration of 1% by weight of the ester oil portion and 5-ethyl-10,10-diphenylphenazasiline at a concentration of 1% by weight of the ester oil portion. The composition of the alkali metal salt portion is set forth in the following Table X.

These embodiments are made by admixing the components thereof at 50-90° C. Table X also contains typical data obtained in testing for oxidative stability samples of these embodiments, of the ester oil portion alone and of the ester oil portion with the arylamine antioxidant portion plus the metal salts indicated in Table X. The test employed is the 425° F. AF Oxidation Test.

TABLE X

| Example No. | Alkali Metal Salt Portion |                                                    |                                                                     | 425° F. AF Oxidation Test Results |                                     |               |
|-------------|---------------------------|----------------------------------------------------|---------------------------------------------------------------------|-----------------------------------|-------------------------------------|---------------|
|             | Component(s)              | Concentration, percent by wt. of ester oil portion | Equivalent metal concentration, percent by wt. of ester oil portion | Oxidation time in hours           | Viscosity in centistokes at 100° F. | Acid No.      |
|             | None                      |                                                    |                                                                     | 0<br>40                           | 14.88<br>59.40                      | 0.03<br>7.50  |
| 79          | Sodium stearate           | 0.128                                              | 0.01—Na                                                             | 0<br>120                          | 14.99<br>19.53                      | 0.03<br>0.87  |
| 80          | Potassium stearate        | 0.08                                               | 0.01—K                                                              | 0<br>120                          | 14.93<br>17.50                      | 0.04<br>0.54  |
|             | Magnesium stearate        | 0.24                                               | 0.01—Mg                                                             | 0<br>40                           | 15.10<br>40.98                      | 0.04<br>7.16  |
|             | Calcium stearate          | 0.15                                               | 0.01—Ca                                                             | 0<br>40                           | 15.00<br>53.07                      | 0.04<br>8.32  |
|             | Barium stearate           | 0.05                                               | 0.01—Ba                                                             | 0<br>40                           | 14.91<br>59.59                      | 0.04<br>8.92  |
|             | Barium stearate           | 0.10                                               | 0.02—Ba                                                             | 0<br>20                           | 14.97<br>42.75                      | 0.03<br>8.25  |
|             | Beryllium stearate        | 0.61                                               | 0.01—Be                                                             | 0<br>40                           | 15.21<br>65.96                      | 0.04<br>10.06 |
|             | Aluminum stearate         | 0.36                                               | 0.01—Al                                                             | 0<br>40                           | 15.11<br>96.73                      | 0.03<br>6.84  |
|             | Cadmium stearate          | 0.07                                               | 0.01—Cd                                                             | 0<br>40                           | 14.96<br>67.73                      | 0.03<br>8.73  |
|             | Zinc stearate             | 0.11                                               | 0.01—Zn                                                             | 0<br>40                           | 15.03<br>33.95                      | 0.04<br>7.29  |
|             | Vanadium stearate         | 0.19                                               | 0.01—V                                                              | 0<br>20                           | 15.02<br>161.52                     | 0.04<br>14.53 |
|             | Iron stearate             | 0.18                                               | 0.01—Fe                                                             | 0<br>20                           | 15.02<br>119.04                     | 0.04<br>10.73 |
|             | Nickle stearate           | 0.12                                               | 0.01—Ni                                                             | 0<br>40                           | 15.01<br>46.84                      | 0.03<br>6.22  |

These data of Table X show that of the metal salts of stearic acid only the alkali metal salts of stearate acid appear to activate arylamine antioxidants at temperatures above 300° F. Hence, the alkali metal salts of the invention generally appear to occupy a unique position relative to arylamine antioxidants generally when employed in synthetic ester oil.

Other features, advantages and specific embodiments of this invention will occur to those in the exercise of ordinary skill in the art after reading the foregoing disclosures. In this connection, while specific embodiments of this invention have been described in considerable detail, variation and modifications of them can be effected without departing from the spirit and scope of the invention as disclosed and claimed.

We claim:

1. A normally liquid composition useful as a lubricant which consists essentially of (a) a synthetic ester oil portion and (b) at a protective concentration a mixture consisting essentially of (1) an arylamine antioxidant portion consisting essentially of an arylamine selected from the group consisting of diphenylamines, N-phenylnaphthylamines, diphenylphenazasilines and (2) an alkali metal salt portion consisting essentially of at least one alkali metal salt selected from the group consisting of alkali metal salts of hydrocarbon carboxylic acids, alkali metal salts of an imide-amide reaction product of a hydrocarbon aminocarboxylic acid and an alkyl amine, alkali metal salts of carboxy terminated polyesters and alkali metal salts of hydroxy aromatic compounds selected from the group consisting of naphthols and hydroxyanthraquinones, the concentration of the alkali metal salt portion being such that the alkali metal concentration is in a range from about 0.001 to about 0.5% by weight of said synthetic ester oil portion and the weight ratio of alkali metal to said arylamine antioxidant portion about 1:30 to about 1:1000.

2. A normally liquid composition useful as a lubricant, which consists essentially of (a) a synthetic ester oil portion and (b) at a concentration in a range from about 0.2 to above 10% by weight of said synthetic ester oil portion a mixture consisting essentially (1) an arylamine antioxidant portion consisting essentially of an arylamine selected from the group consisting of diphenylamines, N-phenylnaphthylamines, diphenylphenazasilines and (2) an alkali metal salt portion consisting essentially of at least one alkali metal salt selected from the group consisting of alkali metal salts of hydrocarbon carboxylic acids, alkali metal salts of an imide-amide reaction product of a hydrocarbon aminocarboxylic acid and an alkyl amine, alkali metal salts of carboxy terminated polyesters and alkali metal salts of hydroxy aromatic compounds selected from the group consisting of naphthols and hydroxyanthraquinones, the concentration of the alkali metal salt portion being such that the alkali metal concentration is in the range from about 0.001 to about 0.5% by weight of said synthetic ester oil portion and the weight ratio of alkali metal to said arylamine antioxidant portion is in a range from about 1:30 to about 1:1000.

3. A normally liquid composition useful as a lubricant, which consists essentially of (a) a synthetic ester oil portion consisting essentially of at least one normally liquid, synthetic ester and (b) at a concentration in a range from about 0.5 to about 5% by weight of said synthetic ester oil portion a mixture a consisting essentially of (1) an arylamine antioxidant portion consisting essentially of at least one arylamine antioxidant selected from the group consisting of diphenylamines, N-phenylnaphthylamines, diphenylphenazasilines, phenothiazines, phenylenediamines and (2) an alkali metal salt portion consisting essentially of at least one alkali metal salt selected from the group consisting of alkali metal salts of hydrocarbon carboxylic acids, alkali metal salts of the imide-amide reaction products of a hydrocarbon amino-

65  
70  
75

carboxylic acid and an alkylamine, alkali metal salts of carboxy terminated polyesters and alkali metal salts of hydroxy aromatic compounds selected from the group consisting of naphthols and hydroxyanthraquinones, the concentration of said alkali metal salt portion being such that the alkali metal concentration is in a range from about 0.005 to about 0.5% by weight of said synthetic ester oil portion and the weight ratio of alkali metal to said arylamine antioxidant portion is in a range from about 1:30 to about 1:1000.

4. A normally liquid composition useful as a lubricant, which consists essentially of (a) a synthetic ester oil portion consisting essentially of 2-butyl-2-ethyl-1,3-propanediol dipelargonate and (b) at a concentration in a range from about 0.5 to about 5% by weight of said synthetic ester oil portion a mixture consisting essentially of (1) an arylamine antioxidant portion consisting essentially of at least one arylamine antioxidant selected from the group consisting of diphenylamines, N-phenylnaphthylamines, dinaphthylamines, phenothiazines, phenylenediamines and diphenylphenazasilines and (2) an alkali metal salt portion consisting essentially of at least one alkali metal salt selected from the group consisting of alkali metal salts of hydrocarbon carboxylic acids, alkali metal salts of the imide-amide reaction product of a hydrocarbon aminocarboxylic acid and an alkylamine, alkali metal salts of carboxy terminated polyesters and alkali metal salts of hydroxy aromatic compounds selected from the group consisting of naphthols and hydroxyanthraquinones, the concentration of said alkali metal salt portion being such that the alkali metal concentration is in a range from about 0.005 to about 0.5% by weight of said synthetic ester oil portion and the weight ratio of alkali metal to said arylamine antioxidant portion is in a range from about 1:30 to about 1:1000.

5. A composition according to claim 4 wherein said arylamine antioxidant portion consists essentially of N-phenyl-1-naphthylamine and 5-ethyl-10,10-diphenylphenazasiline.

6. A composition according to claim 5 wherein said alkali metal salt portion consists essentially of an alkali metal salt of an imide-amide reaction product made by cooking at a temperature of 190-220° C. until an acid number in a range from about 10 to about 150 is obtained a mixture consisting essentially of at least one hydrocarbon aminocarboxylic acid and at least one C<sub>1</sub>-C<sub>18</sub> aliphatic primary amine at a mole ratio of acid to amine in the range from about 1:2 to about 1:4, whereby an imide-amide reaction product is formed and then neutralizing the reaction product to at least 90% of its acidity with at least one alkali metal hydroxide.

7. A composition according to claim 6 wherein said aminocarboxylic acid is ethylenediamine tetraacetic acid and said alkali metal hydroxide is potassium hydroxide.

8. A composition according to claim 4 wherein said arylamine antioxidant portion is selected from the group consisting of an octyldiphenylamine or an octylated styrenated diphenylamine product.

9. A composition according to claim 8 wherein said alkali metal salt portion consists of at least one alkali metal salt of a naphthenic acid.

10. A normally liquid composition useful as a lubricant which consists essentially of (a) a synthetic ester oil portion consisting essentially of trimethylolpropane triheptanoate and (b) at a concentration in a range from about 0.5 to about 5% by weight of said synthetic ester oil portion a mixture consisting essentially of (1) an arylamine antioxidant portion consisting essentially of at least one arylamine antioxidant selected from the group consisting of diphenylamines, N-phenylnaphthylamines, dinaphthylamines, phenothiazines, phenylenediamines and diphenylphenazasilines and (2) an alkali metal salt portion consisting essentially of at least one alkali metal salt selected from the group consisting of alkali metal salts of hydrocarbon carboxylic acids, alkali metal salts of the imide-amide reaction product of a hydrocarbon aminocarboxylic acid and an alkyl amine, alkali metal salts of carboxy terminated polyesters and alkali metal salts of hydroxy aromatic compounds selected from the group consisting of naphthols and hydroxyanthraquinones, the concentration of said alkali metal salt portion being such that the weight ratio of alkali metal to said arylamine antioxidant portion is in a range from about 1:30 to about 1:1000.

imide-amide reaction product of a hydrocarbon amino-carboxylic acid and an alkylamine, alkali metal salts of carboxy terminated polyesters and alkali metal salts of hydroxy aromatic compounds selected from the group consisting of naphthols and hydroxyanthraquinones, the concentration of said alkali metal salt portion being such that the alkali metal concentration is in a range from about 0.005 to about 0.5% by weight of said synthetic ester oil portion and the weight ratio of alkali metal to said arylamine antioxidant portion is in a range from about 1:30 to about 1:1000.

11. A composition according to claim 10 wherein said arylamine antioxidant portion consists essentially of N-phenyl-1-naphthylamine and 5-ethyl-10,10-diphenylphenazasiline.

12. A composition according to claim 11 wherein said alkali metal salt portion consists essentially of the sodium salt of neotridecanoic acid.

13. A normally liquid composition useful as a lubricant, which consists essentially of (a) a synthetic ester oil portion consisting essentially of pentaerythritol tetra(mixed pelargonate/2-ethylhexanoate) and (b) a concentration in the range from about 0.5 to about 5% by weight of said synthetic ester oil portion a mixture consisting essentially of (1) an arylamine antioxidant portion consisting essentially of at least one arylamine antioxidant selected from the group consisting of diphenylamines, N-phenylnaphthylamines, dinaphthylamines, phenothiazines, phenylenediamines and diphenylphenazasilines and (2) an alkali metal salt portion selected from the group consisting of alkali metal salts of hydrocarbon carboxylic acids, alkali metal salts of the imide-amide reaction product of a hydrocarbon aminocarboxylic acid and an alkyl amine, alkali metal salts of carboxy terminated polyesters and alkali metal salts of hydroxy aromatic compounds selected from the group consisting of naphthols and hydroxyanthraquinones, the concentration of said alkali metal salt portion being such that the alkali metal concentration is in a range from about 0.005 to about 0.5% by weight of said synthetic ester oil portion and the weight ratio of alkali metal to said arylamine antioxidant portion is in a general range from about 1:30 to 1:1000.

14. A composition according to claim 13 wherein said arylamine antioxidant portion consists essentially of p,p'-dioctyldiphenylamine.

15. A composition according to claim 14 wherein said alkali metal salt consists essentially of at least one alkali metal salt of a naphthenic acid.

16. An antioxidant composition useful for synthetic ester lubricants, which comprises a mixture consisting essentially of (1) an arylamine antioxidant portion consisting essentially of at least one arylamine antioxidant selected from the group consisting of diphenylamines, N-phenylnaphthylamines, dinaphthylamines, phenothiazines, phenylenediamines, and diphenylphenazasilines and (2) as a high temperature activator for said arylamine antioxidant portion an alkali metal salt portion consisting essentially of at least one alkali metal salt selected from the group consisting of alkali metal salts of hydrocarbon carboxylic acids, alkali metal salts of the imide-amide reaction product of a hydrocarbon aminocarboxylic acid and an alkyl amine, alkali metal salts of carboxy terminated polyesters and alkali metal salts of hydroxy aromatic compounds selected from the group consisting of naphthols and hydroxyanthraquinones, the concentration of said alkali metal salt portion being such that the weight ratio of alkali metal to said arylamine antioxidant portion is in a range from about 1:30 to about 1:1000.

17. A composition according to claim 16 wherein said arylamine antioxidant is a diphenylamine selected from the group consisting of diphenylamine, p-octyldiphenylamine or p,p'-dioctyldiphenylamine.

18. A composition according to claim 16 wherein said arylamine antioxidant portion includes 5-ethyl-10,10-diphenylphenazasiline.

19. A composition according to claim 16 wherein said arylamine antioxidant in said arylamine portion is selected from the group consisting of an octylated diphenylamine product or an octylated styrenated diphenylamine product.

20. A composition according to claim 16 wherein said arylamine antioxidant is a dinaphthylamine selected from the group consisting of dinaphthylamine or di-2-naphthylamine.

21. A composition according to claim 16 wherein said arylamine antioxidant is a phenothiazine selected from the group consisting of phenothiazine or N-ethylphenothiazine.

22. A composition according to claim 16 wherein said alkali metal salt portion consists essentially of at least one alkali metal salt of a hydrocarbon carboxylic acid selected from the group consisting of a naphthenic acid or an aliphatic carboxylic acid having 1 to 18 carbon atoms.

23. A composition according to claim 16 wherein said alkali metal salt portion consists essentially of at least one alkali metal salt of an imide-amide reaction product made by cooking at a temperature of 190-220° C. until an Acid No. in the range from about 10 to about 150 is obtained a mixture consisting essentially of at least one hydrocarbon aminocarboxylic acid and at least one C<sub>1</sub>-C<sub>18</sub> aliphatic primary amine at a mole ratio of acid to amine in the range from about 1:2 to about 1:4, whereby an imide-amide reaction product is formed, and neutralizing said reaction product to at least 90% of its acidity with at least one alkali metal hydroxide.

24. An antioxidant composition useful in synthetic ester lubricants which comprises a mixture consisting essentially of (1) an arylamine antioxidant portion consisting essentially of at least one arylamine antioxidant selected from the group consisting of diphenylamines, N-phenylnaphthylamines, dinaphthylamines, phenothiazines, phenylenediamines, and diphenylphenazasilines and (2) as a high temperature activator for said arylamine antioxidant portion an alkali metal salt of an imide-amide reaction product made by cooking at a temperature of 190-220° C. until an Acid No. in a range from about 10 to about 150 is obtained a mixture con-

sisting essentially of at least one hydrocarbon aminocarboxylic acid and at least one C<sub>1</sub>-C<sub>18</sub> aliphatic primary amine at a mole ratio of acid to amine in the range from about 1:2 to about 1:4, whereby an imide-amide reaction product is formed and neutralizing said reaction product to at least 90% of its acidity with at least one alkali metal hydroxide.

25. An antioxidant composition useful in synthetic ester lubricants which comprises the mixture consisting essentially of (1) an arylamine antioxidant portion consisting essentially of N-phenyl-1-naphthylamine and 5-ethyl-10,10-diphenylphenazasiline and (2) as a high temperature activator for said arylamine antioxidant portion an alkali metal salt of an imide-amide reaction product made by cooking at a temperature of 190-220° C. until an acid number in a range from about 10 to about 150 is obtained a mixture consisting essentially of at least one hydrocarbon aminocarboxylic acid and at least one C<sub>1</sub>-C<sub>18</sub> aliphatic primary amine at a mole ratio of acid to amine in the range from about 1:2 to about 1:4, whereby an imide-amide reaction product is formed and neutralizing said reaction product to at least 90% of its acidity with at least one alkali metal hydroxide.

25

#### References Cited

##### UNITED STATES PATENTS

|           |         |                 |       |            |
|-----------|---------|-----------------|-------|------------|
| 2,001,108 | 5/1935  | Parker          | ----- | 252-39 X   |
| 2,079,051 | 5/1937  | Sullivan et al. | ----- | 252-18     |
| 2,321,577 | 6/1943  | Clayton et al.  | ----- | 252-49.7 X |
| 2,344,988 | 3/1944  | Kavanagh et al. | ----- | 252-42.7   |
| 2,954,342 | 9/1960  | Hotten          | ----- | 252-42.1 X |
| 3,053,768 | 9/1962  | Cupper          | ----- | 252-56 X   |
| 3,115,519 | 12/1963 | Crouse et al.   | ----- | 252-56 X   |
| 3,126,344 | 3/1964  | Matuszak et al. | ----- | 252-56 X   |

#### OTHER REFERENCES

Barnes et al., "Synthetic Ester Lubricants," Petroleum Engineering, August 1957, pp. 454-458.

40

DANIEL E. WYMAN, Primary Examiner.

P. P. GARVIN, Assistant Examiner.